

# United States Patent

[19]

Nishizawa et al.

[11] 3,880,677

[45] Apr. 29, 1975

[54] **METHOD FOR PRODUCING A SINGLE CRYSTAL OF  $IN_xGA_{1-x}P$**

[75] Inventors: **Jun-Ichi Nishizawa; Ken Suto; Yasuo Okuno**, all of Sendai, Japan

[73] Assignee: **Zaidan Hojin Handotai Kenkyu Shinkokai**, Sendai-shi, Japan

[22] Filed: **Dec. 27, 1972**

[21] Appl. No.: **318,884**

[52] U.S. Cl. .... **156/624; 148/171; 148/172; 75/134 T; 252/62.3 GA**

[51] Int. Cl. .... **H01L 7/38**

[58] Field of Search .... **148/1.6, 171-173; 75/134 T; 252/62.3 GA**

[56] **References Cited**

UNITED STATES PATENTS

- |           |         |                        |             |
|-----------|---------|------------------------|-------------|
| 3,278,342 | 10/1966 | John et al. ....       | 148/1.6     |
| 3,414,441 | 12/1968 | Gershenzon et al. .... | 252/62.3 GA |
| 3,614,549 | 10/1971 | Lorenz et al. ....     | 148/171 X   |
| 3,628,998 | 12/1971 | Blum et al. ....       | 148/171     |

OTHER PUBLICATIONS

Scifres et al., *Physical Review B*, Vol. 5, No. 6, Mar. 15, 1972, pp. 2206-2215.

Logan et al., *Journal of Applied Physics*, Vol. 42, No. 6, May 1971, pp. 2328-2335.

Hakki et al., *Journal of Applied Physics*, Vol. 41, No. 13, Dec. 1970, pp. 5291-5296.

Primary Examiner—G. Ozaki  
Attorney, Agent, or Firm—Craig & Antonelli

[57]

**ABSTRACT**

A single crystal of  $IN_xGA_{1-x}P$  ( $0 < x < 0.9$ ) having the desired  $1-x$  value is produced when an In melt including P whose mole ratio to In is less than about 0.2 and Ga whose mole ratio to P is between  $\frac{1}{2}(1-x)M_p$  and  $2(1-x)M_p$ , wherein  $M_p$  is mole ratio of P to In in the In melt is heated at a temperature higher than a solidus temperature which ranges from 800°C. to 1150°C. of a single crystal of  $IN_xGA_{1-x}P$  to be obtained for 10 hours to 20 hours, and cooled to a room temperature or some practical temperature higher than the room temperature at a cooling rate of about 2°C/hour to about 50°C/hour.

10 Claims, 2 Drawing Figures



FIG. 1



FIG. 2



**METHOD FOR PRODUCING A SINGLE CRYSTAL  
OF  $\text{In}_x\text{Ga}_{1-x}\text{P}$**

The present invention relates to a method for producing a single crystal of  $\text{In}_x\text{Ga}_{1-x}\text{P}$ , more particularly to a method for producing  $\text{In}_x\text{Ga}_{1-x}\text{P}$  by utilizing a liquid phase epitaxial method.

Single crystals of  $\text{In}_x\text{Ga}_{1-x}\text{P}$  have recently attracted much interest since they are useful for light-emitting diodes which emit efficient radiation up to the green portion of the visible spectrum.

Generally, single crystals of  $\text{In}_x\text{Ga}_{1-x}\text{P}$  are grown by a liquid phase epitaxial method in which In is used as a melt.

It is, however, difficult to obtain single crystals of  $\text{In}_x\text{Ga}_{1-x}\text{P}$  having a desired value of  $x$ .

For controlling the value of  $x$  in the single crystals of  $\text{In}_x\text{Ga}_{1-x}\text{P}$  in the paper of "Elaboration et propriétés optiques d'alliages  $\text{Ga}_x\text{In}_{1-x}\text{P}$ " by H. Rodot et al., in *Comptes Rendus De L'Academie Des Sciences*, Vol. 269 B, (September 1969) pp. 381-384, P is diffused into a In-Ga melt, and in the paper of "Electroluminescent Properties of InGaP grown by LPE on GaAs" by B.W. Hakki, in 137 National Meeting of Electrochemical Society, Los Angeles (1970), Abstract No. 74, pp. 204-206, the molar ratios of InP and GaP which are provided as the source of P and Ga are controlled.

An object of the present invention is to provide a novel method for producing a single crystal of  $\text{In}_x\text{Ga}_{1-x}\text{P}$  wherein  $0 < 1-x < 0.9$ , i.e.,  $x$  is greater than 0.1 and less than 1.0, by utilizing the liquid phase epitaxial method.

Another object of the present invention is to provide a method for producing a single crystal of  $\text{In}_x\text{Ga}_{1-x}\text{P}$  ( $0 < 1-x < 0.9$ ) having the desired  $x$  value ( $0.1 < x < 1$ ).

A further object of the present invention is to provide a method for producing a single crystal of  $\text{In}_x\text{Ga}_{1-x}\text{P}$  ( $0 < 1-x < 0.9$ ) wherein the  $x$  value is easily controlled.

For obtaining the above-mentioned objects, in the present invention, the mole ratio  $M_{Ga}$  of Ga to P in the In melt is controlled between  $\frac{1}{2}(1-x)M_p$  and  $2(1-x)M_p$  in the In melt, wherein  $M_p$  is the mole ratio of P to the In in the In melt, for obtaining  $\text{In}_x\text{Ga}_{1-x}\text{P}$ , and wherein  $0 < M_p < 0.2$ .

These and other objects and advantages of the present invention will become apparent to those skilled in the art from a consideration of the following specification and claims, taken in conjunction with the accompanying drawings in which:

FIG. 1 shows a sectional view of an apparatus wherein  $\text{In}_x\text{Ga}_{1-x}\text{P}$  according to the present invention is obtained; and

FIG. 2 is a diagram showing a relationship between the  $1-x$  value of  $\text{In}_x\text{Ga}_{1-x}\text{P}$  obtained by the present invention and the mole ratio of Ga to P in the In melt.

A crystal,  $\text{In}_x\text{Ga}_{1-x}\text{P}$ , having desired value of  $1-x$  is obtained, when a quartz ampoule 1, wherein In melt 2, a certain amount of phosphorous 3 whose mole ratio to In( $M_p$ ) is less than about 0.2, and a certain amount of Ga4 whose mole ratio  $M_{Ga}$  to P in the In melt is controlled between (when the mole ratio of P in the In melt is  $M_p$ ),  $\frac{1}{2}(1-x)M_p$  and  $2(1-x)M_p$  are introduced is disposed in a quartz tube 5 disposed in a furnace 6, and the quartz ampoule 1 is heated at a temperature higher than a solidus temperature which ranges from 800°C. to 1150°C. of a single crystal of  $\text{In}_x\text{Ga}_{1-x}\text{P}$  to be obtained by the furnace 6 for from about 10 hours to

about 20 hours, and is cooled to a room temperature at a cooling rate of from about 2°C/hour to about 50°C/hour. It will be understood that the single crystal may be cooled from a temperature between about 200°C. from the solidus temperature to room temperature, i.e., about 25°C.

When the amount of In, P and Ga are 4.000 gr., 0.140 gr., and 0.200 gr., respectively, single crystals of  $\text{In}_x\text{Ga}_{1-x}\text{P}$  having a value of 0.660, 0.665, 0.655 and 0.699 for  $1-x$  are obtained. And also, when the amount of In, P and Ga are 4.000 gr., 0.140 gr. and 0.315 gr., respectively, single crystal of  $\text{In}_x\text{Ga}_{1-x}\text{P}$  having 0.76 as a value of  $1-x$  is obtained.

Numerous experiments were conducted by the present inventors and the results of the experiments are shown in FIG. 2.

In FIG. 2, a vertical direction shows the  $1-x$  value of  $\text{In}_x\text{Ga}_{1-x}\text{P}$ , and a horizontal direction shows mole  $M_{Ga}$  of Ga to P in the In melt.

As apparent from FIG. 2, when mole  $M_{Ga}$  of Ga to P in the In melt is controlled between  $\frac{1}{2}(1-x)M_p$  and  $2(1-x)M_p$ , wherein  $M_p$  is mole ratio of P to In in the In melt, a single crystal of  $\text{In}_x\text{Ga}_{1-x}\text{P}$  having desired value of  $1-x$  can be obtained. And also, it is apparent that, for obtaining single crystals of  $\text{In}_x\text{Ga}_{1-x}\text{P}$  having desired value of  $1-x$ , a preferable range of mole ratio  $M_{Ga}$  of Ga is between  $\frac{1}{4}(1-x)M_p$  and  $(3/2)(1-x)M_p$ , and especially between  $\frac{1}{8}(1-x)M_p$  and  $(5/4)(1-x)M_p$ .

However, when  $1-x$  value of  $\text{In}_x\text{Ga}_{1-x}\text{P}$  is over 0.9, that is,  $x$  is less than 0.1, the above-mentioned relationship between mole ratio  $M_{Ga}$  of Ga to P in the In melt and mole ratio  $M_p$  of P to In is not suitable. Therefore, the present invention is suitable for a method for producing single crystals of  $\text{In}_x\text{Ga}_{1-x}\text{P}$  wherein the range of  $1-x$  value is more than 0 but less than 0.9.

In the above-mentioned embodiment, though the single crystal of  $\text{In}_x\text{Ga}_{1-x}\text{P}$  is obtained in a closed tube, that is, in the quartz ampoule, it is understood that the present invention is applicable to another type of liquid phase epitaxial method, such that, a method wherein In melt including Ga and P is contacted with a seed material, such as GaAs and GaP, heated at a temperature lower than that of the In melt. It will be appreciated that the temperature of the In melt should be kept at a temperature higher than a temperature ranging from 800°C. to 1150°C. (the solidus temperature of the desired crystal) which temperature of the melt is dependent on the single crystal to be obtained. The difference in temperature may be several degrees, e.g., 5° to 50°.

While the invention has been explained in detail, it is to be understood that the technical scope of the present invention is not limited to that of the foregoing embodiment but applicable to all liquid phase epitaxial methods as stated in the claims.

What is claimed is:

1. A method for producing a single crystal of  $\text{In}_x\text{Ga}_{1-x}\text{P}$  wherein  $0 < 1-x < 0.9$ , comprising the steps of: preparing an In melt; introducing P so that its mole ratio to In in the melt is less than about 0.2 into the In melt; introducing Ga whose mole ratio to P in the In melt is between  $\frac{1}{2}(1-x)M_p$  and  $2(1-x)M_p$  wherein  $M_p$  is mole ratio of P to In in the In melt, into the In melt; heating the In melt including P and Ga at a temperature higher than a solidus temperature of a single

crystal of  $In_xGa_{1-x}P$  to be obtained, for a period of from about 10 hours to about 20 hours; and cooling the resultant In melt to room temperature at a cooling rate of about  $2^{\circ}\text{C}/\text{hour}$  to about  $50^{\circ}\text{C}/\text{hour}$ .

2. A method for producing a single crystal of  $In_xGa_{1-x}P$  according to claim 1, wherein the mole ratio of Ga to P in the In melt is between  $\frac{3}{4}(1-x)M_p$  and  $(3/2)(1-x)M_p$ .

3. A method for producing a single crystal of  $In_xGa_{1-x}P$  according to Claim 1, wherein the mole ratio of Ga to P in the In melt is between  $\frac{7}{8}(1-x)M_p$  and  $(5/4)(1-x)M_p$ .

4. A method for producing a single crystal according to claim 1, which further comprises the steps of introducing said In melt, P and Ga into an ampoule, and closing said ampoule prior to heating the In melt including P and Ga.

5. A method for producing a single crystal according to claim 1, wherein the In melt including P and Ga is heated in a closed container.

6. A method for producing a single crystal of  $In_xGa_{1-x}P$  wherein  $0 < 1-x < 0.9$ , comprising the steps of: preparing an In melt; introducing P so that its mole ratio to In in the melt is less than about 0.2, into the In melt; introducing Ga so that its mole ratio to P in the In melt is between  $\frac{1}{2}(1-x)M_p$  and  $2(1-x)M_p$  wherein  $M_p$  is the mole ratio of P to In in the In melt, into

5

15

10

20

25

30

In melt;

disposing the In melt including P and Ga in a furnace; disposing a seed material at a different portion in the furnace from the portion at which In melt is disposed;

heating the In melt including Ga and P at a temperature higher than a solidus temperature of a single crystal of  $In_xGa_{1-x}P$  to be obtained, for about 10 hours to about 20 hours;

heating the seed material at a temperature lower than that of In melt;

contacting the In melt with the seed material; and cooling the In melt to a room temperature at a cooling rate of about  $2^{\circ}\text{C}/\text{hour}$  to about  $50^{\circ}\text{C}/\text{hour}$ .

7. A method for producing a single crystal of  $In_xGa_{1-x}P$  according to claim 6, wherein the mole ratio of Ga to P in the In melt is between  $\frac{3}{4}(1-x)M_p$  and  $(3/2)(1-x)M_p$ .

8. A method for producing a single crystal of  $In_xGa_{1-x}P$  according to claim 6, wherein the mole ratio of Ga to P in the In melt is between  $\frac{7}{8}(1-x)M_p$  and  $(5/4)(1-x)M_p$ .

9. A method for producing a single crystal according to claim 6, wherein the seed material is GaAs or GaP.

10. A method for producing a single crystal according to claim 6, wherein the mole ratio  $M_p$  of P to In in the In melt is greater than 0.

\* \* \* \* \*

35

35

40

45

50

55

60

65